

## UNITED STATES PATENT OFFICE

1,935,266

## METALLIC DENTAL FILLING COMPOSITION

Friedrich Hauptmeyer, Essen, Germany

No Drawing. Application December 22, 1928,  
Serial No. 328,056, and in Germany March 1,  
1928

## 1 Claim. (Cl. 106—6)

This invention relates to a plastic composition to be used for filling carious teeth. The object of the invention is to provide a composition of this kind which can be polished well, 5 which possesses high resistance to wear, and which is neutral to chemical agents. This object is obtained according to the invention by making a mixture of a chemically neutral chromium-nickel iron or steel alloy in powdered condition and a dental cement, the proportions being 10 preferably determined so that there is just sufficient of the metallic alloy to insure the desired high resistance to wear and good polishability.

15 Any of the known chemically neutral chromium-nickel iron alloys, or chromium-nickel steel alloys may be used, and they may contain other components not jeopardizing the advantageous property of chemical neutrality. As examples of the alloys which may be used, reference is made to the patents to Benno Strauss, No. 1,339,378, Friedrich Hauptmeyer, No. 1,421,776, and Harry Etchells, No. 1,522,813.

The dental filling composition may be produced, for example, in the following manner. Finely powdered chemically neutral chromium-nickel steel containing about 20 percent of chromium and 7 percent of nickel is mixed with one of the cements used in dental surgery, with 30 addition of the usual setting liquid, and a paste which is at first plastic, but which concretes later on is made thereof. The lower limit of the percentage of chromium-nickel steel is determined by tests showing whether the mixture 35 still possesses the desired high resistance to wear and good polishability. In a mass serving for the purpose set forth, this percentage is about 50. This paste is filled while still in plastic state into the cavity of the tooth and tamped.

After the cement has set, the plug is polished and then forms a tooth filling which is both chemically neutral toward all agents that come into consideration, and highly resistant to wear, and is far superior to amalgam filling which under certain circumstances is not harmless. 60

The manner in which the alloys are brought into the powdered condition is of no importance for the present invention. They may be pulverized by means of mills such as those described 65 in the patents to C. T. Fuller, No. 1,041,769 and E. Podszus, No. 1,573,017. A still better procedure, based upon certain particular properties of the chemically neutral chromium-nickel iron and steel alloys, is as follows: A piece of chemically 70 neutral chromium-nickel iron or steel alloy is heated for a considerable time to a temperature between 500 to 900° C., after which it is subjected to the attack of a suitable corrosive, such as dilute sulphuric acid containing copper sulphate. The heating causes the separation from the austenitic matrix of the alloy of carbides, which are segregated in the grain boundaries, from which they are substantially washed out 75 by the action of the corrosive agent. Under the influence of this inter-crystalline corrosion the alloy first loses its metallic ring, then becomes like leather, so that it can be bent and crumbled in the fingers. In this condition the alloy can easily be reduced to an extremely fine powder 80 and this is advantageous because the polishability of the composition depends upon the fineness of the metal particles. 85

I claim:

A dental filling mass consisting of a mixture 90 of about 50% of dental cement and about 50% of a powdered chromium-nickel iron or steel alloy neutral to chemical agents.

FRIEDRICH HAUPTMEYER.

40

95

45

100

50

105

55

110